

Nov. 21, 1950

G. W. JERNSTEDT

2,530,967

BRIGHT ALLOY PLATING

Filed Sept. 9, 1947



WITNESSES:

Robert Chard  
Rev. G. Groome

INVENTOR

George W. Jernstedt.  
BY  
Frederick Shapoe  
ATTORNEY

## UNITED STATES PATENT OFFICE

2,530,967

## BRIGHT ALLOY PLATING

George W. Jernstedt, Pittsburgh, Pa., assignor to  
Westinghouse Electric Corporation, East Pitts-  
burgh, Pa., a corporation of Pennsylvania

Application September 9, 1947, Serial No. 772,977

2 Claims. (Cl. 204—44)

1

This invention relates to electro-plating and, more particularly, to electro-plating of bright ternary alloy coatings upon metal surfaces to provide for appearance and corrosion-resistance.

This application is a continuation-in-part of my copending patent applications Serial No. 458,399, filed September 15, 1942, and entitled "Bright Alloy Plating," now abandoned, Patent No. 2,435,967, issued February 17, 1948, entitled "Bright Alloy Plating," and Serial No. 591,073, filed April 30, 1945, now abandoned.

In applying electro-plated coatings to metal surfaces in order to provide for attractive appearance and predetermined color and corrosion-resistance, only a limited number of metals are ordinarily available. Of these, some are costly and their use is limited for this reason. At the present time, certain of the more usual electro-plating metals are scarce, and the number of electro-plating metals available to the industry for general use has been sharply reduced. It is quite important to employ metals obtainable at low prices which are not so scarce for plating purposes, and a feature of this invention is to provide desirable bright plate by using metals obtainable in relative abundance.

As is well known to those skilled in the art, no bright electro-plated metal coating is satisfactory to a high degree in meeting to a high degree all the major plated coating requirements such as high corrosion-resistance, low cost, abrasion-resistance, and bright, attractive surface color. Some metals, for instance chromium, when applied by plating do not confer any significant degree of corrosion-resistance to the base metal, and it is necessary to apply protective coatings such as nickel plating or copper plating between the chromium plate and the base metal. Other metals such as silver, are subject to rapid tarnishing or oxidation and, therefore, are undesirable for many commercial purposes.

A feature of my invention is the economical electro-deposition of a bright silvery coating of a ternary alloy of copper, tin and zinc having as its outstanding properties high corrosion-resistance and high abrasion resistance. This optimum combination of characteristics is not available in any other known metal or alloy.

Ternary alloy plating has been practiced in some cases but, in general, the electro-plating of alloys consisting of three or more components is ordinarily quite difficult. Not only are the conditions of the electrolyte extremely critical as a rule, but changes in voltage and amperage per unit area of anode or cathode are reflected in dis-

2

proportionate changes in the results. However, according to this invention, an easily controlled ternary alloy plating method is an important feature. The ternary alloy is plated directly from anodes of the alloy, thereby greatly reducing the cost of the plating operation. Relatively great variations in the bath and other plating conditions are tolerable without undue detrimental results following.

10 The object of this invention is to provide a process for producing an electro-plated ternary alloy coating upon the surfaces of metal which coating is characterized by a silvery bright, attractive surface appearance, good abrasion-resistance, and an extraordinarily high degree of corrosion-resistance without the use of other protective coatings.

Another object of this invention is to provide for electro-plating a bright silvery ternary alloy 20 coating from anodes composed of the alloy.

Other objects of the invention will, in part, be obvious and will, in part, appear hereinafter. For a fuller understanding of the nature and objects of this invention, reference should be had to the 25 following detailed description and drawing, the single figure of which is a cross-section of an electro-plating apparatus functioning according to the invention.

Pursuant to this invention, a ternary alloy composed of copper, tin, and zinc is electro-plated upon metal members with highly satisfactory results. By varying the composition of anodes of the alloy and the operating conditions of the apparatus a bright silvery electroplated coating, similar to chromium or silver plate, is produced. In either case, the electro-plating may be conducted within a relatively wide range of operating conditions with complete success.

It has been proposed heretofore to plate copper, zinc, and tin as a bright silvery alloy from a bath or electrolyte containing suitable salts of these metals using insoluble anodes. However, the preparation of the metal in the form of salts and the fact that the salts produce a much smaller amount of plated metal than the weight of the salts renders the cost of the prior art practice excessive. A further disadvantage present in such prior art practice is due to the fact that the bath containing only metal salts continually varies as the electroplating, proceeds, producing an increasing excess proportion of the anion of the metal salt as well as depleting the metal content thereby producing a continually varying bath. This leads to non-uniform plating, besides 55 requiring continual maintenance of the bath.

From a commercial standpoint, the prior art practice is not satisfactory or economical.

The ternary alloy which is electro-deposited in practicing the present invention preferably consists of from 50% to 75% copper, 15% to 30% tin, and 5% to 20% zinc, all parts by weight. The presence of minor amounts of other metals or impurities is believed not to affect the nature of the electro-plated product. Particularly good results are obtained if the copper content is from 55% to 65%, the tin from 20% to 30% and the zinc from 10% to 20%. The tin content of the anodes may be two or three per cent more than the plated alloy, since a small fraction of the tin precipitates out of the electrolyte. Therefore, the anodes may contain from 15% to 35% tin, the copper being from 50% to 75% and the zinc from 5 to 20%.

In making the anodes, it has been found that the ternary alloy is conveniently prepared by melting the required weight of copper in a crucible with the predetermined amount of tin and zinc added just prior to the casting of the melt into suitable anodes. Alternately, a brass of suitable composition may be melted initially and tin added in producing the ternary alloy. Permanent molds or, in some cases, sand molds may be used in casting anodes. During the casting operation, supporting hooks of a conducting metal such as steel may be cast into the anodes to provide for supporting them from the anode conductor bar in the electro-plating apparatus. In case a conductor anode frame or holder is to be employed, the ternary alloy may be cast into any desired shape, such as balls, suitable for putting into the anode holder.

Referring to the single figure of the drawing, there is illustrated one form of electro-plating apparatus 10 suitable for the practice of the invention. The apparatus 10 comprises a tank 12 of wood, steel, or other chemically resistant material capable of retaining a cyanide electrolyte 14 therein. A suitable source of heat such, for example as a steam coil 28, is provided for the tank 12 since the preferred operating temperature is above room temperatures. The electrolyte 14 consists of the following constituents:

|                                                                                          | Ounces per gal. |
|------------------------------------------------------------------------------------------|-----------------|
| Free cyanide                                                                             | 0.5 to 5.0      |
| Copper                                                                                   | 0.2 to 0.50     |
| Tin                                                                                      | 0.05 to 0.20    |
| Zinc                                                                                     | 0.1 to 0.5      |
| Sodium carbonate                                                                         | 2.0 to 12.0     |
| Sodium hydroxide, about 0.25 to 0.8 ounce per gallon to give a pH of from about 12 to 13 |                 |

When the composition is maintained within the limits indicated, plating may be accomplished with satisfactory results. To secure an electro-plating bath of the above-composition, the following chemicals in the indicated quantities by weight may be added per 1000 parts of water:

|                  | Parts    |
|------------------|----------|
| Copper cyanide   | 2 to 5   |
| Sodium cyanide   | 10 to 80 |
| Zinc cyanide     | 1 to 6   |
| Sodium stannate  | 3/4 to 4 |
| Sodium carbonate | 15 to 90 |

and sufficient sodium hydroxide (roughly 3 to 6 parts) to give a pH of from 12 to 13.5.

An electrolyte that has been satisfactory for

both barrel and still-tank plating has the following composition:

|                                                                         | Ounces per gallon |
|-------------------------------------------------------------------------|-------------------|
| Copper cyanide                                                          | 0.5               |
| Zinc cyanide                                                            | 0.27              |
| Sodium stannate ( $\text{Na}_2\text{SnO}_3 \cdot 3\text{H}_2\text{O}$ ) | 0.22              |
| Sodium cyanide                                                          | 3.75              |
| Sodium carbonate                                                        | 4.0               |
| Sodium hydroxide                                                        | 0.6               |

The electrolyte, when maintained in a pH range of from about 12.6 to 13.5, produces excellent bright silvery electroplate. The anodes were composed of from 52% to 65% copper, 25% to 35% tin and 10% to 20% zinc. Analysis of the ternary alloy electro-plate produced by this last electrolyte in combination with the anodes shows copper from 55% to 60%, tin 25% to 28% and zinc 14% to 18%.

In all of the above compositions zinc may be added as zinc sulfate. Other zinc, tin and copper salts, which are soluble in a cyanide solution may be employed in preparing the electrolyte. It will be understood that potassium salts may be used instead of sodium salts, allowance being made for the difference in molecular weight. The electrolyte is prepared by dissolving the finely powdered salts in the predetermined quantity of water. The solution may be filtered before introducing it into the tank 12.

The anodes 18 prepared as indicated previously are suspended or supported from the anode bars 16. From a cathode bar 20 a cathode supporting member 22 is suspended. In plating small articles, such as shown at 24 in the figure, it may be desirable to provide the cathode member 22 with a plurality of hooks or supports 26, only a portion of which comprises exposed metal for flow of electrical current to the articles supported thereon. The remainder of the cathode support may be coated with a suitable electrically insulating material to prevent wastage of current. When members 24, which are to be plated, are suspended on the supports 26, electrical contact will be made between the members and the exposed metal portions on the support. In other cases where the members being plated are of sufficiently large size, they may be suspended directly from the cathode bar 20 by using suitable conducting hooks or the like.

The electrolyte 14 is extremely reactive with the metal of the anodes 18. The anode efficiency is about 100% while the cathode efficiency is about 35%, thereby the metal content of the bath tends to approach the limits of concentration set forth in the first table. Accordingly, it is necessary under most conditions to employ one or more relatively insoluble steel or carbon anodes in combination with a number of ternary alloy anodes 18. Satisfactory results have been obtained with from 15% to 30% of the total anode area consisting of the alloy anodes, the remaining anode area being provided by the insoluble anodes.

In order to plate bright silvery deposits on the members 24 in the apparatus 10, it has been found necessary to apply a voltage between the anodes 18 and members 24 critically correlated with the separation between centers. In ordinary plating tanks where the anode to cathode distance is standardized at from 6 to 8 inches, the voltage should be maintained within the limits of from 3 to 5 volts. For this 6 to 8 inch spacing, if the voltage is substantially above 5 volts milky deposits are produced, while with a voltage of sub-

stantially less than 3 volts yellow deposits plate out. For distances between anode and cathode other than from 6 to 8 inches, it has been discovered that the voltage should be increased in the proportion of 1 volt for each 4 inches increase in spacing and decreased in the proportion of 1 volt for each 4 inches decrease in spacing. At a one inch separation, about the minimum practically feasible, from 1½ to 2 volts will electrodeposit a bright silvery alloy plate.

The alloy plating baths operated as disclosed herein have outstanding throwing power. It compensates for the uneven distances between bulky articles and the anodes. The throwing power enables crevices of great depth to plate as brightly as the surface. In many cases sections of tubing will plate bright entirely over both inside and outside surfaces.

*Example I*

Steel pole blocks in shape being approximately cubes with a concave hollow in one face, of a dimension of approximately 1½ inches on each edge, previously plated with 0.0005 inch of copper, were mounted on a rack in groups of 48 and placed in a still tank containing an electrolyte of the following composition:

|                                       | Ounces per gal. |
|---------------------------------------|-----------------|
| Cyanide (free) -----                  | 2.0             |
| Metal:                                |                 |
| Copper -----                          | 0.32            |
| Zinc -----                            | 0.13            |
| Tin -----                             | 0.08            |
| Sodium carbonate -----                | 5.0             |
| Sodium hydroxide to give a pH of 12.8 |                 |
| Temperature 150° F.                   |                 |

The anodes were spaced 7 inches from the center of the pole blocks. The anodes were comprised of 75% in area of steel and 25% in area of an alloy composed of copper 56%, tin 28% and zinc 16%. Electrical current at 4 volts was applied to the anodes and cathodes, the current density being approximately 15 amperes per square foot. A silvery bright ternary alloy plate 0.0002 inch thick was deposited in 23 minutes. The composition of the electrodeposited plate was copper 57%, tin 26% and zinc 17%.

*Example II*

A plating barrel was loaded with threaded instrument terminals composed of copper. The terminals were from 1 inch to 1¼ inches long and of a diameter of ¼ inch. About 50 pounds of the terminals were placed in the barrel. The barrel was rotated at an oblique angle to the vertical in a tank containing the following electrolyte:

|                                       | Ounces per gal. |
|---------------------------------------|-----------------|
| Cyanide (free) -----                  | 3.0             |
| Metal:                                |                 |
| Copper -----                          | 0.35            |
| Zinc -----                            | 0.15            |
| Tin -----                             | 0.10            |
| Sodium carbonate -----                | 5.0             |
| Sodium hydroxide to give a pH of 12.8 |                 |
| Temperature 155° F.                   |                 |

The anodes were disposed at the outside of the barrel at an average distance of nine inches from the surface of the mass of the terminals in the barrel. The anodes comprised 75% insoluble anodes and 25% soluble anodes of the same composition as in Example I. Current at 5½ volts was applied. In an hour the parts were plated with 0.0002 inch of a bright ternary alloy having

the same composition as the plate in Example I.

In producing bright smooth deposits of the silvery plate, it has been found that derivatives of alpha, beta, and gamma betaines containing at least one non-cyclic hydrocarbon radical composed of from 10 to 20 carbon atoms may be added to the electrolyte 14 as anti-pitting and brightening agents. The amount of betaine may be added in amounts ranging from 0.01 to 1 ounce per gallon to produce the desired results.

The apparatus may be operated at a temperature of 140° F. to 160° F. over a wide range of amperes per unit area. Still tank plating has been accomplished at temperatures of 140° F. to 150° F., while barrel plating operates well at 150° F. to 160° F. It is possible to obtain ternary alloy coatings 0.0001 to 0.0005 inch thick in a short time, about 12 minutes at a current density of 15 amperes per square foot is required per 0.0001 inch thickness of deposit. For most purposes, coatings of this thickness have adequate covering power and corrosion-resistance. In some cases where it is desirable to have a thicker coating, plates varying from 0.001 to 0.002 inch thick and even heavier and which are quite bright have been obtained by electro-plating for greater periods of time.

The electro-plated alloy is surpassed only by freshly plated silver in reflectivity. Tests indicate that its reflectivity is approximately 85% of that of freshly plated silver. However, an advantage over silver plate is that the ternary alloy plate deteriorates in reflectivity very slowly, whereas silver becomes tarnished rapidly under normal circumstances.

The corrosion-resistance of the ternary alloy electro plate is superior to nickel, tin, chromium, and silver when these latter metals are plated on copper or copper alloys. For example, 0.001 inch thickness of nickel on copper when subjected to salt-spray tests will fail in less than 100 hours. The ternary alloy 0.0002 inch thick plated on copper regularly passes a 200 hour salt-spray test without any visible corrosion. Very few electro-plated metals have the corrosion-resistance that the ternary alloy of this invention has.

An additional advantage of the ternary alloy applied to copper, in particular, is that the alloy can be soldered to as effectively and easily as to tinned parts. This feature is exceedingly important in the fabrication of instruments, meters, and other electrical apparatus, for example, where contacts and other parts must be soldered in assembling the apparatus. It is essentially non-magnetic and therefore is useful in instrument manufacture.

The alloy may be plated upon many metals used as a base. Steel and ferrous metals may be directly plated; though, to secure maximum corrosion resistance, steel is initially copper or brass plated and then ternary alloy plated. Copper, brass and other copper alloys are excellent bases for the alloy plate.

Hardness tests indicate that the ternary alloy electro-plate is much harder and more resistant to abrasion than electro-plated coatings of nickel, tin, or silver.

A particular advantage of the alloy plating bath described herein over the usual bright plating baths is due to the greatly superior throwing power of the ternary alloy. The alloy has a greater throwing power than nickel, tin, silver, or chromium. For this reason, the ternary alloy coatings need only be about one-fifth as thick as a nickel, tin, or silver plate to give a good cover-

age and corrosion-resistance to metal surfaces. Since certain changes in carrying out the above processes and certain modifications in the compositions which embody the invention may be made without departing from its scope, it is intended that all the matter contained in the above description or shown in the accompanying drawing shall be interpreted as illustrative and not in a limiting sense.

I claim as my invention:

1. The method of electrodepositing bright silvery corrosion-resisting coatings of a ternary alloy composed of from 50% to 75% copper, 15% to 30% tin and 5% to 20% zinc upon a member which comprises making the member the cathode in an aqueous electrolyte comprising essentially 0.5 to 5 oz. of free cyanide per gallon, 0.2 to 0.5 oz. of copper per gallon, 0.05 to 0.2 oz. of tin per gallon, 0.1 to 0.5 oz. of zinc per gallon, alkali metal hydroxide and 2 to 12 oz. of alkali metal carbonate per gallon, the electrolyte being maintained at a temperature of between approximately 140° F. and 160° F. and at a pH of from 12 to 13.5 the anode comprising a ternary alloy composed of from 50% to 75% copper, 15% to 35% tin and 5% to 20% zinc and passing electrical current through the electrolyte at a potential proportional to the distance between the anode and the cathode, the potential being from 3 to 5 volts between the anode and cathode when they are spaced 6 to 8 inches apart, and the voltage being increased or decreased one volt for each 4 inches increase or decrease, respectively, in the spacing between anode and cathode.

2. The method of electrodepositing bright silvery corrosion-resisting coatings of a ternary alloy composed of from 52% to 65% copper, 20% 35

to 30% tin, and 10% to 20% zinc upon a member which comprises making the member the cathode in an aqueous electrolyte comprising essentially 0.5 to 5 oz. of free cyanide per gallon, 0.2 to 0.5 oz. of copper per gallon, 0.05 to 0.2 oz. of tin per gallon, 0.1 to 0.5 oz. of zinc per gallon, alkali metal hydroxide and 2 to 12 oz. of alkali metal carbonate per gallon, the electrolyte being maintained at a temperature of between approximately 140° F. and 160° F. and at a pH of above 12, the anode comprising a ternary alloy composed of from 52% to 65% copper, 25% to 35% tin and from 10% to 20% zinc and passing electrical current through the electrolyte at a potential proportional to the distance between the anode and cathode, the potential being from 3 to 5 volts between the anode and cathode when they are spaced 6 to 8 inches apart, the voltage being increased or decreased one volt for each 4 inches increase or decrease, respectively, spacing between anode and cathode.

GEORGE W. JERNSTEDT.

#### REFERENCES CITED

25 The following references are of record in the file of this patent:

#### UNITED STATES PATENTS

| Number    | Name      | Date          |
|-----------|-----------|---------------|
| 2,181,773 | Wernlund  | Nov. 28, 1939 |
| 2,198,365 | Cinnamon  | Apr. 23, 1940 |
| 2,255,057 | Holt      | Sept. 9, 1941 |
| 2,435,967 | Jernstedt | Feb. 17, 1948 |

#### FOREIGN PATENTS

| Number | Country       | Date    |
|--------|---------------|---------|
| 22,002 | Great Britain | of 1906 |